

FIP8309      XR      1,959,406  
CATION OF TEXTILES & FIBERS, [REDACTED]

1,959,406

May 22, 1934

## UNITED STATES PATENT OFFICE

1,959,406

## TREATMENT OF TEXTILE

Emanuel Brooks, Brooklyn, N. Y.

No Drawing. Application November 12, 1932,  
Serial No. 642,461

4 Claims. (Cl. 8—20)

The present invention relates to a textile treating process, and it particularly relates to a process for pre-shrinking textiles of cotton or similar materials.

5 As is widely known, cotton textile products, particularly washable garments made of cotton, tend to shrink and decrease in size incident to each washing and cleansing operation. This shrinkage frequently continues over long periods of time and 10 as a result the cotton garment or clothing article decreases in size to such a degree that it must be discarded by the possessor thereof.

Many attempts have been made to shrink cotton goods or garments before retail sale, and although 15 partial pre-shrinking is widely attained, a complete pre-shrinking has not been readily commercially achieved. Such complete shrinking processes involve drastic chemical treatments and processing which not only were expensive but 20 often resulted in deterioration of the textile material.

An object of the present invention is to provide a pre-shrinking process for cotton piece goods which will assure substantially complete 25 pre-shrinking of such goods on a commercially economical basis without drastic chemical treatments.

Other objects will appear during the course of the following specification.

30 It has been found that if a relatively small amount of ammonium alum and sodium bisulphite are utilized in the pre-shrinking bath extraordinary surprising results are obtained. Although ammonium alum or ammonium aluminum sulphate will cause a slight shrinking of cotton piece goods when utilized by itself, when sodium bisulphite is included, this shrinking becomes surprisingly complete without any noticeable deterioration of the piece goods. The sodium bisulphite in 40 addition to catalyzing the action of the ammonium alum on the piece goods also may be utilized for its bleaching effect in certain instances, with the result that simultaneous shrinking and bleaching are possible. Exactly what causes this most advantageous combined action of ammonium alum and sodium bisulphite is not readily apparent, but it must be something closely tied up with the properties and character of the cellulose fiber constituting the base of the cotton material.

50 Although the composition of the bath may be widely varied, in one instance it has been found very satisfactory to utilize 20 parts of water, 2 parts of ammonium alum and 1 part of sodium bisulphite. This composition may be conveniently varied so that there will be between 1 to 4 ounces

of ammonium alum and  $\frac{1}{4}$  to 3 ounces of sodium bisulphite utilized to from 10 to 50 ounces of water.

A striking advantage residing in the process of the present invention resides in the fact that it is only necessary to heat the bath to a temperature approaching boiling for a relatively short period. In one example, the cotton piece goods was satisfactorily processed when heated in the bath to 180 to 190° F. and after a two hour soaking. However, the temperature of treatment may be varied from 150 to 210° F. and from 1 to 10 hours as may be found most desirable.

After soaking, the material is removed from the bath, the liquids are removed by pressing and/or centrifuging and are then dried. Although generally not included in the preferred processes, other alums may be substituted for ammonium alum in certain cases as may also certain other reducing sulphur acids, such as sodium sulphite and/or sodium hydrosulphite.

In general, baths containing aluminum sulphate or alums when combined with reducing sulphur acid salts, appear to have the most satisfactory effects.

It is obvious that the above described invention may be widely varied in details and many different embodiments thereof may be devised. It is therefore intended that the invention may be only restricted by the scope of the appended claims.

## What is claimed is:

1. A process of pre-shrinking cotton piece goods which comprises immersing them in a bath containing dissolved ammonium alum and sodium bisulphite.

2. A process of pre-shrinking cotton piece goods which comprises immersing them in a heated bath containing ammonium alum and sodium bisulphite for from 1 to 6 hours.

3. A process of pre-shrinking cotton piece goods which comprises subjecting the material to treatment in a bath containing 20 parts of water, 2 parts of ammonium alum, and 1 part of sodium bisulphite, heating the bath to 180 to 190° F., continuing the soaking for two hours and then removing the piece goods from the bath and drying them.

4. A pre-shrinking bath for cotton textile materials comprising an aqueous solution containing 20 parts of water, 2 parts of ammonium alum and 1 part of sodium bisulphite.

EMANUEL BROOKS.

110